

1

3,248,186  
FLOW CHARACTERISTICS OF WAXY  
PETROLEUM RESIDUUM

Darrell Brownawell, Scotch Plains, and Harold N. Miller, Plainfield, N.J., assignors to Esso Research and Engineering Company, a corporation of Delaware  
No Drawing. Filed Sept. 12, 1962, Ser. No. 223,252  
3 Claims. (Cl. 44—62)

This invention is concerned with the preparation and utilization of acyl polystyrenes having  $C_{20+}$  acyl side chains attached to the polystyrene nucleus as blending agents for improving the flow characteristics of very high wax-containing petroleum residual oils typified by the residuum of a North African crude known as Zelten, or similar petroleum oils, that boil above 650° F. and have pour or flow points above 75° F.

A typical Zelten residuum, which boils above 680° F., contains about 20 wt. percent wax and has a flow point of 105° F. This wax includes waxes of relatively high molecular weight ranging from about  $C_{30}$  to  $C_{50}$  paraffins which gives rise to a number of problems in transporting and storing this kind of heavy oil. Even though this kind of oil has a relatively low viscosity as measured by conventional methods compared to heavy oils of low wax content, the handling of the high wax content residuum creates special difficulties on account of the manner in which the oil undergoes changes in flow characteristics on being subjected to changes in temperature. Generally, the standardized ASTM pour point is reasonably indicative of how low the temperature of an oil can be decreased to the point at which it can be satisfactorily made to flow. However, with high waxy residua, such as a Zelten oil, the pour points determined by the standardized procedure are variable and a function of prior thermal treatment. Thus, it was found necessary to alter the standard ASTM pour point procedure to obtain a reproducible and more meaningful measure of flow characteristics in testing the high wax-containing residual oils, such as in Zelten crude residuum. In this flow point test, a sample of oil is first heated to 200° F., then cooled to 32° F. before it is again heated to an intermediate temperature in the range of 90° to 200° F. for testing under the standard ASTM procedure. By putting the oil through a temperature cycle series, such as mentioned, a determination is made of the flow point corresponding to the maximum pour point in the series, and such a flow point is the best measure so far achieved in determining how well such oils can be kept fluid in storage and for pumping or transporting.

In making the discovery of the present invention, a number of conventional pour point depressing compounds, such as shown in the prior art for use in lubricating oils and distillate oils, were tried and found to be quite unsuitable. Such conventional pour point depressants are typified by polymer compounds such as chlorinated wax-naphthalene condensation polymers made from waxes having varying carbon chains varying from about 16 to 24 carbon atoms, acyl polystyrenes in which the acyl group contains fewer than 18 carbon atoms, alkylated polystyrenes having as many as 22 carbon atoms in the alkyl group, and polyvinyl stearate. While some of the aforementioned polymers give some lowering of the flow point in the high wax-containing residua using the ordinary ASTM pour point method or even a single heating treatment, they were found to be unsuitable when the oil was put through a second thermal cycle which involved re-heating the oil containing the additive to various temperatures up to temperatures of 200° F.

In accordance with the present invention, a surprisingly enhanced flow point characteristic was found to be given

2

to the high wax-containing residual oils by blending with these oils certain small amounts of acyl polystyrenes having 20 to 22 carbon atoms in the acyl group, the acyl group thus approximating arachidic and behenic acids in length, i.e.  $CH_3(CH_2)_{18}COOH$  and  $CH_3(CH_2)_{20}COOH$ , and mixtures thereof. It was determined also important to use concentration ranges of this kind of acyl polystyrene, and preferably from 0.1 to 1.0 wt. percent, for the best results.

10 In general, polyacylated polystyrenes are assigned the following structure:



15 wherein the acyl group



20 is defined as containing a straight chain alkyl group R of at least 19 carbon atoms, and subscript n is a number from 2 to 50 of the recurring units of the acylated polystyrene. For the purposes of the present invention, the 25 acyl group



30 which makes the acyl polystyrene potent for improving the flow characteristics of a high wax-containing residual 35 contains at least 20 up to 30 carbon atoms, and preferably 20 to 22 carbon atoms. It appears that these particular compounds have never before been produced.

The method of forming these acyl polystyrenes comprises 40 dissolving commercial polystyrene in o-dichlorobenzene and adding to this solution 0.5 to 1.0 mole of a carboxylic acid chloride-aluminum chloride complex. The ratio of styrene units to acyl units in the acyl polystyrene can vary 45 from 1:1 to 2:1. This complex is formed by mixing equimolar amounts of aluminum chloride with the carboxylic acid chloride dissolved in o-dichlorobenzene at a temperature of 20° to 70° C. After all the acid chloride-aluminum chloride complex has been added to the solution of the polystyrene and hydrogen chloride 50 evolution has stopped, the aluminum catalyst is destroyed by addition of water or alcohol to the reaction mixture. The acylated polystyrene is then taken up in a suitable hydrocarbon solvent, such as heptane or kerosene, and washed with an aqueous alkaline solution and water. 55 The solvent may be evaporated to isolate the polymer or the polymer may be dissolved in the solvent for blending with the residual oil.

The high molecular weight acylating reactants that are 60 of particular interest and use for the purpose of the present invention are the  $C_{20}$  and  $C_{22}$  acid chlorides, or mixtures including these two acid chlorides, obtained from straight chain carboxylic acids, such as arachidic and behenic acid, or commercial acid mixtures including these two. These acid chlorides are obtained by treating 65 the corresponding acid dissolved in a suitable solvent, such as o-dichlorobenzene, with chlorinating agents, such as phosphorus trichloride. The reaction temperature is maintained at 20 to 80° C.

It was found that in order to achieve proper dispersion 70 of the acyl polystyrenes in the high boiling and high wax-containing residua, that the blending and mixing should take place with the oil heated to an elevated temperature

in the range of 100° F. to about 250° F., to melt the waxes and thus obtain homogeneous dispersion. In determining the flow points of the blends, duplicate tests were made; each blend was put through at least two thermal cycles to find out whether the change in flow

proved in flow properties, is a premium oil as compared to other crude residua which have much lower pour points. This is illustrated by a comparison of the Zelten waxy oil with crude petroleum residua known as Aramco and Kuwait.

TABLE II  
Processing Zelten crudes

|                                   | Heavy Fuel Oil Inspections |        |        |        |
|-----------------------------------|----------------------------|--------|--------|--------|
|                                   | Zelten                     | Aramco | Kuwait | Target |
| Vol. percent 680° V. VT+ on crude | 35                         | 39     | 47     | —      |
| Inspections on 680° F. VT+:       |                            |        |        |        |
| Gravity, ° API                    | 22                         | 15     | 14     | —      |
| Sulfur, wt. percent               | 0.4                        | 3.0    | 4.2    | 13.5   |
| Viscosity, SF @ 122° F            | 65                         | 110    | 340    | 40-175 |
| MNI, wt percent                   | 2.3                        | 4.0    | 3.8    | 17     |
| Conradson carbon, wt. percent     | 4.5                        | 8.9    | 10-11  | —      |
| Flow pt., ° F.                    | 105                        | 65     | 55     | 175    |
| Hot filtration sed., wt percent   | 0.01                       | 0.02   | 0.02   | 10.15  |

<sup>1</sup> maximum.

point was stable. In the first thermal cycle, the blend 25 is heated first to 200° F., cooled to 32° F., reheated to 200° F., and then cooled. To determine the flow point in the second thermal cycle, the blend is heated to 200° F., cooled to 32° F., reheated to 115° F. and then cooled to the flow point. The comparisons on the effects of the 30 additives on the flow points of the high wax-containing residuum are shown below:

TABLE I  
Effect of additives on flow points of 680° F.+ virgin Zelten residuum

| Additive                                                | Additive wt. percent conc. | ° F., Lower flow <sup>1</sup> | ° F., Upper flow <sup>2</sup> |
|---------------------------------------------------------|----------------------------|-------------------------------|-------------------------------|
| 680° F.+Virgin zelten residuum                          | None                       | 95                            | 100                           |
|                                                         | None                       | 100                           | 100                           |
| C <sub>18</sub> Acyl polystyrene                        | 1.0                        | 75                            | 75                            |
|                                                         | 0.1                        | 100                           | 100                           |
|                                                         | 1.0                        | 45                            | 65                            |
| C <sub>20</sub> Acyl polystyrene                        | 0.3                        | 50                            | 55                            |
|                                                         | 0.1                        | 60                            | 65                            |
|                                                         | 2.0                        | 65                            | 65                            |
| C <sub>22</sub> Acyl polystyrene                        | 1.0                        | 55                            | 60                            |
|                                                         | 0.3                        | 55                            | 55                            |
|                                                         | 0.1                        | 75                            | 85                            |
|                                                         | 1.0                        | 65                            | 70                            |
| Mixed C <sub>20</sub> -C <sub>22</sub> acyl polystyrene | 0.3                        | 60                            | 65                            |
|                                                         | 0.1                        | 65                            | 75                            |
| Wax-naphthalene condensate (from 135° F., M.P. wax)     | 1.0                        | 100                           | 105                           |
|                                                         | 0.3                        | 100                           | 105                           |
|                                                         | 0.1                        | 100                           | 100                           |
| Wax-naphthalene condensate (from 180° F., M.P. wax)     | 1.0                        | 65                            | 100                           |
|                                                         | 0.3                        | 55                            | 100                           |
|                                                         | 0.1                        | 55                            | 100                           |
| C <sub>22</sub> Alkyl polystyrene                       | 1.0                        | 90                            | 90                            |
|                                                         | 0.3                        | 100                           | 100                           |
|                                                         | 0.1                        | 95                            | 95                            |
|                                                         | 1.0                        | 100                           | 100                           |
| Polyvinyl stearate                                      | 0.3                        | 100                           | 100                           |
|                                                         | 0.1                        | 100                           | 105                           |

<sup>1</sup> Lower flow point thermal cycle, 200° F.-32° F.-200° F.-lower flow point.

<sup>2</sup> Upper flow point thermal cycle, 200° F.-32° F.-115° F.-upper flow point.

It can be seen from the data in the above table that outstanding desired results in lowering the flow point of the residual oils are obtained, particularly by using the C<sub>20</sub> acylated polystyrene and the C<sub>22</sub> acylated polystyrene additives. All the other additives showed a flow point reversion or ineffectiveness in the repeated reheating and 65 recooling of the blends.

Further studies on the blends showed that there is a critical concentration of the C<sub>20</sub> acylated polystyrene and C<sub>22</sub> acylated polystyrene within the range of 0.1 to 1.0 wt. percent at which concentration, there appears to occur the formation of stable aggregates of the additive with wax in the oil if the blending and mixing of the additive has been properly carried out.

The Zelten residuum boiling above 680° F., which typifies the kind of high wax-containing oils to be im-

70 able products, such as straight chain olefins. The column under the notation "Target" indicates types of blends which it is desired to make using the Zelten residuum as a blending stock provided one can lower the flow point. For example, it is desired to mix the Zelten crude in a 50/50 mixture with the Aramco or Kuwait residuum. Of course, such a blending lowers the wax content, but even so, the flow point may not be sufficiently reduced without using the specially adapted C<sub>20</sub>+ acyl polystyrenes as additives in suitable concentration for lowering the flow point back to below the 75° F. target. For example, in the 50/50 Zelten/Aramco blend, the addition of only 0.15 wt. percent of C<sub>22</sub> acyl polystyrene was found sufficient to meet the target of a 75° F. flow point, the 50/50 mixture without this additive having a flow point of 95° F. Thus, the proportion of additive with

respect to the Zelten residuum in the blend is 0.3 wt. percent. In other words, the concentration of the  $C_{20}$  + acyl polystyrene additive required for the desired improvement of fluidity can be based on the proportion of the high wax-containing oil component.

The invention described is claimed as follows:

1. A petroleum residuum oil composition having improved characteristics, which comprises essentially a high wax content petroleum residuum boiling above about 650° F. and having a flow point and a pour point above 75° F., improved with respect to its flow characteristics by incorporating and blending therewith an amount of about 0.1 to 1.0 wt. percent of  $C_{20}$  to  $C_{22}$  acyl polystyrene having the acyl group



wherein R is a straight chain alkyl group containing from 19 to 21 carbon atoms, the number of styrene units in the acyl polystyrene is 2 to 50, and the ratio of styrene units to acyl units present in the acyl polystyrene varies from 1:1 to 2:1.

2. Oil composition as defined by claim 1 wherein the amount of acyl polystyrene present is in the range from 0.1 to 0.3% by weight.

3. An improved composition of petroleum crude oil containing high melting paraffins of 30 to 50 carbon atoms per molecule and having a natural flow-point above 75° F. to which has been added a minor proportion, not exceeding 1% by weight and sufficient to lower the flow-point of said oil below 75° F., of a  $C_{22}$ - $C_{22}$  acyl polystyrene having the acyl group



10 wherein R is a straight chain alkyl group containing from 19 to 21 carbon atoms, the number of styrene units in the acyl polystyrene is 2 to 50, and the ratio of styrene 15 units to acyl units present in the acyl polystyrene varies from 1:1 to 2:1.

#### References Cited by the Examiner

##### UNITED STATES PATENTS

|    |           |         |              |         |
|----|-----------|---------|--------------|---------|
| 20 | 2,642,398 | 6/1953  | Butler       | 252—52  |
|    | 2,703,817 | 3/1955  | Serniuk      | 260—592 |
|    | 3,069,245 | 12/1962 | Wythe et al. | 44—62   |

25 DANIEL E. WYMAN, Primary Examiner.